

## UNITED STATES PATENT OFFICE

ORIN D. CUNNINGHAM, OF INDIANAPOLIS, INDIANA, ASSIGNOR TO PETER C. REILLY,  
OF INDIANAPOLIS, INDIANA

## FROTH FLOTATION PROCESS

No Drawing. Application filed September 10, 1928, Serial No. 305,143. Renewed February 19, 1931.

This invention relates to the froth flotation process for the recovery of ores and minerals and has for its object the use of a certain class of organic substances in the concentration of such ores and minerals.

The present invention is based on the discovery that the xanthogenates of certain alcohol-like cyclic and heterocyclic compounds are very effective flotation collecting reagents. Certain ring-structured organic compounds possess the property of reacting with alkali metal hydroxides and carbon disulfide to form xanthogenates, said organic compounds can be characterized by being hydrogenated completely or almost completely to saturation, and by the presence of a hydroxyl group, such for example, as hexa-hydro-phenol (cyclo-hexanol), the hexa-hydro-cresols (methyl-cyclo-hexanol), tetra-hydro-beta-naphthol, terpineol, menthol, borneol and all other like substances that may be regarded as hydrogenated hydroxy-aromatic derivatives.

The hydrogenation of hydroxy-aromatic compounds is necessary in order to enable them to enter into the xanthogenate reaction since phenol and the cresols, for example, do not enter into reaction with an alkali metal hydroxide and carbon disulfide, as do their corresponding hydrogenated derivatives, cyclohexanol and the methyl cyclohexanols respectively; this difference in chemical behavior being due to the fact that the hydrogenation of unsaturated (benzenoid structured) aromatic compounds transforms them to saturated (or more completely saturated) compounds possessing aliphatic-like properties, hydrogenation thereby imparting to hydroxy-aromatic compounds (phenol, cresols, and the like) the property, characteristic of the aliphatic alcohols (alkyl hydroxy-compounds), of reacting with alkali metal hydroxide and carbon disulfide to form xanthogenates, although not to such a pronounced degree. Accordingly, the hydrogenated hydroxy-aromatic compounds are commonly called cyclic or heterocyclic alcohols, a class of substances distinguished from the true aliphatic alcohols by their ring structure.

Since alcohol-like properties are to some extent imparted to hydroxy-aromatic compounds when they are only partially saturated with hydrogen, as for example the di and tetrahydro derivatives of phenol the cresols and the like, it is not desired to limit the classification of the compounds of this invention that form active xanthogenate flotation reagents to the completely hydrogenated compounds, but to include also the hydrogenated hydroxy-aromatic derivatives of any degree of hydrogenation, such as di, tetra, and hexahydro compounds, etc.

The cyclic alcohols being very good frothing agents (as set forth in a companion application, Serial No. 305,142 filed concurrently herewith), the preparation of the xanthogenate collecting reagent of this invention may very conveniently be made up in such proportions as to have present in the preparation an excess of the cyclic alcohol to serve as a frothing agent, the resulting product thus serving both as a collecting and frothing reagent.

As specific examples, the following methods are given for preparing the cyclic and heterocyclic alcohol xanthogenate flotation reagents of this discovery, without restricting the invention to these examples.

## Example 1

8.3 parts of the hydrogenated cresols (O, M, P mixed) and 2.9 parts of sodium hydroxide were thoroughly ground together in a mortar at the temperature of a steam bath for about 15 minutes and after cooling, 5.5 parts of carbon disulfide ( $CS_2$ ) were added and the grinding continued (more  $CS_2$  being added as it evaporated) until the reaction was complete, as shown by the constancy of the weight. These proportions are the theoretical for completely converting the hydrogenated cresols to the xanthogenate compound and under the conditions of this preparation about 75% of the carbon disulfide entered into reaction. The product of reaction was then dried under a vacuum at room temperature in the presence of a drying agent, and then ground into a powder.

*Example 2*

8.3 parts of hydrogenated cresols were reacted with 0.57 parts of sodium hydroxide (NaOH) by grinding together at the temperature of a steam bath until a smooth paste was obtained, cooling, and then reacting with 1.1 parts of carbon disulfide as above until the maximum amount had entered into reaction; this preparation being made up in such a proportion as to give a satisfactory combined frothing and collecting reagent for the ore tested (0.31 lb. of the reagent per ton of dry ore was used). The product was 15 semi-liquid or pasty in consistency.

The invention is not restricted to the conditions or proportions or materials, of the above preparations, but may use a lower temperature such as room temperature for carrying out the first step in the preparation, or instead of carrying out the reaction in two steps, the reacting substances (hydrogenated cresols, alkali and CS<sub>2</sub>) may be ground together in a one step operation, other alkalies can be used as well as other hydrogenated hydroxy-aromatic bodies, or mixtures thereof.

*Example 3*

For the preparation of a combined frothing and collecting agent from steam distilled pine oil (terpineol or terpene alcohol), 7.36 parts of pine oil and 0.9 parts of sodium hydroxide were ground together at room temperature to a smooth paste, then 1.75 parts of carbon disulfide (CS<sub>2</sub>) was added, and the reaction mixture ground together (with the addition of more CS<sub>2</sub> as it evaporated) until the maximum amount of carbon disulfide had reacted. In all of these reactions there was from 65 to 75% of the theoretical amount of carbon disulfide that entered into reaction. The reaction product was a liquid.

*Example 4*

45 8.3 parts of pine oil, 2.1 parts of sodium hydroxide and 4.0 parts of carbon disulfide were reacted together as above to give a combined frothing and collecting reagent (0.30 lb. of reagent per ton of ore giving very 50 satisfactory recoveries on the ore tested).

In the case of solid cyclic (or heterocyclic) alcohols, like menthol and borneol, the xanthogenate reaction may be carried out as above by first dissolving the alcohol substance in some inert solvent like toluene, treating with alkali metal hydroxide and carbon disulfide (in one or two steps) then vacuum-distilling off the solvent.

In the above examples sodium hydroxide 60 is used in preference to potassium hydroxide because of the greater stability of the flotation reagent formed, but the invention is not restricted to the use of sodium hydroxide alone, nor to the use of the alkali metal hydroxide in the solid form, since in some 65

cases a concentrated alkali metal hydroxide solution in water may be used, or for other preparations metallic sodium may be employed.

The reactions taking place may be explained as follows (using hydrogenated phenol), to the correctness of which theory the invention is not restricted.



The products obtained, as those illustrated in the above examples, were employed in the flotation of a copper sulfide ore of the Utah Copper Co., analyzing about 1.0% copper, in the ratio of about one tenth pound (0.1 lb.) of product per ton of dry ore, and for the products requiring a frothing agent pine oil was used. The ore was subjected to the ordinary flotation operation in a mechanical agitation type of flotation cell, and a lime circuit employed. A tailing analyzing 0.10% copper or under was obtained, together with a high grade concentrate, corresponding to a recovery of about 90% of the copper value in 100 the ore treated.

In other tests both smaller and larger amounts of the reagents of this invention have been employed, in the flotation of ores, with satisfactory results, and the said new reagents have been used both alone and with other flotation reagents, with satisfactory results. Furthermore, the conditions for carrying out a flotation operation may be varied widely from those included in the above examples and any type of flotation machine can be used, or, instead of an alkaline circuit, a neutral or acid circuit can be used.

In the above specification reference has been made to the use of hydrogenated phenol and cresols in the preparation of a satisfactory flotation reagent. It is to be understood that other closely analogous substances, such as hydrogenated tar acid (from either high or low temperature tar) can likewise be employed within the scope of the invention.

*Claims:*

1. A process which comprises froth flotation of ores in the presence of a xanthogenate of a hydrogenated hydroxy-aromatic derivative.
2. A process which comprises froth flotation of ores in the presence of a xanthogenate of a hydrogenated tar acid product.
3. A process which comprises froth flota-

tion of ores in the presence of a xanthogenate of a hydrogenated hydroxy-aromatic derivative together with a hydrogenated hydroxy-aromatic derivative as a frothing agent.

5 4. As a new composition of matter, a mixture comprising a hydrogenated hydroxy-aromatic derivative and a xanthogenate of a hydrogenated hydroxy-aromatic derivative, such composition having collecting and  
10 frothing properties.

In testimony whereof I have signed my name to this specification.

ORIN D. CUNNINGHAM.

15

20

25

30

35

40

45

50

55

60

65